

## UNITED STATES PATENT OFFICE

2,221,559

## PROCESS FOR BLEACHING OILS, FATS AND WAXES

Emil Scheller, Lorsbach in Taunus, Germany, assignor to Deutsche Gold und Silber Scheideanstalt, Frankfurt-on-the-Main, Germany, a corporation of Germany

No Drawing. Application October 20, 1937, Serial No. 170,073. In Germany March 5, 1936

5 Claims. (Cl. 260—423)

This application relates to the bleaching of oils, fats and waxes. In the improved process of bleaching these substances it is proposed to utilize bleaching agents, preferably bleaching agents of the oxidizing type. More particularly, the improved process is concerned with the bleaching of waxes such as commercial beeswax and other waxes in order that a light colored product of especial value in the cosmetic industry may be secured.

10 There are now known to the art various methods for bleaching oils, fats and waxes. For the bleaching of beeswax and other waxes of value in industrial processes, bleaching by subjecting the emulsified wax to the action of an oxidizing bleaching agent has already been disclosed. In these processes the beeswax or other wax being bleached is maintained at a temperature at which it is in the molten condition during the bleaching process. An alkaline medium yielding active oxygen or active chlorine is usually utilized, the bleaching being carried out under conditions wherein the wax and medium form a more or less stable emulsion. However, bleaching with the 15 permanganates as the active agents has also been employed for lightening the color of oils, fats and waxes.

In processes as now utilized in the art it is customary, at the conclusion of the bleaching step 20 wherein the oil, fat or wax in emulsified form is treated with the bleaching agent, to break the emulsion by the addition of an acid to the emulsified mixture. This results in precipitation of the beeswax or other product being treated. The 25 precipitated substance is then ordinarily washed and subjected to a second bleaching operation in the molten or liquid condition. While hydrogen peroxide may frequently be used in the first step, that wherein the emulsified oil, fat or wax 30 is treated with the bleaching agent, it is also frequently utilized as the bleaching agent in the latter step. A process of the general type described is given in full in German Patent 595,126.

Since the improved process utilizes relatively 35 mild chemical reagents it has found distinct favor for industrial operations. When relatively mild chemicals are utilized the wax retains its desirable natural characteristics and is substantially unchanged, except as to color, during the bleaching operations. The absence of substantial 40 change in the character of the wax during bleaching in accordance with the process described is evidenced by the fact that the wax constants are substantially the same at the conclusion of 45 bleaching as prior to bleaching. Moreover, the

waste water resulting from the treatment of the wax is neutral in reaction, thus indicating no substantial decomposition of the wax. Beeswax bleached in accordance with the procedure outlined and more fully described in German patent 595,126 has been found of especial value in industries such as the cosmetic industry, wherein a whiter but substantially unchanged product is desired.

However, it has been observed in some cases 10 that unsatisfactory bleaching is secured when oils, fats and waxes, and more especially beeswax, are subjected to bleaching processes of the general type outlined. At first it was believed that the unsatisfactory bleaching was attributable 15 to the bleaching activity of the agents utilized in the process and to the difficulty of bleaching dark colored organic substances such as the usual commercial waxes and beeswaxes. It has now been found, however, that the unsatisfactory bleaching results from the presence 20 of small amounts of inorganic acids in the product being treated in the subsequent bleaching step wherein the product, in molten form, is subjected to the action of hydrogen peroxide. The 25 presence of inorganic acids in the wax or beeswax, or in the oil or fat, during the hydrogen peroxide bleaching step seriously interferes with bleaching and impairs the character of the resultant product.

As previously pointed out, it is customary at the conclusion of the step wherein the oil, fat or wax 30 is subjected, in emulsified form, to the action of a bleaching agent, to recover the product from the emulsion by the addition of an acid such as 35 sulfuric acid thereto. In present processes the product is then carefully washed several times for the purpose of removing that acid. It has been found that repeated remelting of the product when that product is a solid and repeated washing with water does not remove the last traces 40 of the acid used for breaking the emulsion. Moreover, in practice clarification is only rarely so complete that very distinct separation between the molten wax treated and the aqueous treating 45 agents utilized will result. Depending primarily upon the quality of the wax or other product treated and the apparatus employed, there are usually formed intermediate layers or more or less heavy appearance. These layers are customarily 50 treated together with the liquid wax in the ensuing bleaching step or steps, thus introducing into the wax small amounts of acids which materially interfere with bleaching.

Another source of acid resides in the hydrogen 55

peroxide itself which is employed for the final bleaching step. It must be remembered that commercial hydrogen peroxide contains acid, usually an inorganic acid such as sulfuric or phosphoric acids, and that when commercial hydrogen peroxide is added to the product being treated and maintained in the molten state, in processes such as that described in German Patent 595,126, definite amounts of acid are introduced. This is clearly shown by experimental results for frequently when large amounts of hydrogen peroxide are employed in an attempt to secure improved bleaching results, amounts greater than those normally utilized, it is observed that the bleaching results are less favorable than when the smaller amounts of hydrogen peroxide were employed. This decrease in bleaching activity is attributable to the introduction into the process of larger amounts of acid with the larger amounts of hydrogen peroxide, the greater amount of acid present seriously interfering with bleaching.

I have now found that the second bleaching step of processes such as that described in German Patent 595,126, the step wherein the oil, fat or wax in the liquid or molten state is treated with hydrogen peroxide, may be more successfully carried out with results of greater uniformity if care is taken to insure the substantial absence of free inorganic acids during this portion of the process. The substantial elimination of acids during this bleaching operation may be accomplished in various ways, one of which is by neutralization of the acid present by the addition of materials which are alkaline in reaction.

It is possible to employ for the purpose alkaline agents such as ammonia, caustic soda, alkali metal salts, or alkaline earth metal salts. Specific examples of salts suitable include sodium acetate, sodium carbonate, and lime. I have found, however, that best results are obtained when magnesium oxide is utilized for neutralizing the free acid present. It is especially advantageous to utilize for neutralizing the acid those alkaline agents which, upon neutralization, do not form acid products with the acids that they neutralize. For this reason sodium acetate is not very suitable as an addition agent for neutralizing free acid present in the product being bleached for it forms acetic acid during the neutralization of the inorganic acid present. I prefer to employ alkaline addition agents which form products which are neutral or almost neutral in reaction with the acids that they neutralize. While a slight excess of the alkalinizing agent employed may not be injurious to the oil, fat or wax, it is preferable to add but small amounts of these alkaline agents, amounts not exceeding those sufficient to impart to the resulting mixture during the bleaching operation a pH value between 7 and 8.5. The amount of alkaline agent added should not exceed that necessary to insure a substantially neutral medium, i. e., one having a pH value between 7 and 8.5, during the bleaching step.

I have observed that best results are obtained when magnesium oxide is utilized as the agent for neutralizing the acids present in the oils, fats or waxes or present in the hydrogen peroxide during the step wherein the oil, fat or wax, in liquid or molten form, is treated with hydrogen peroxide. This is probably because magnesium oxide is substantially completely neutral in reaction, and, moreover, yields with the acids neutralized, salts which are neither acid nor basic in reaction. While an excess of magnesium ox-

ide is not injurious to the oil, fat or wax nor does it interfere with the bleaching process, it should, nevertheless, be avoided if possible. I have found it advantageous to employ from 0.1 to 0.2% magnesium oxide, that amount being by weight based upon the weight of the oil, fat or wax being treated.

As an alternative way of accomplishing the same result, I have found it possible to utilize in the final bleaching step hydrogen peroxide to which has been added an alkali metal peroxide in such quantity that the inorganic acid present in the substance being bleached is substantially neutralized. A slight excess of the alkali metal peroxide may be present if desired and enough may be added to render the pH of the resulting solution slightly on the alkaline side. Care should be taken, however, to have present only such amounts of alkali metal peroxide as will not raise the pH of the oil, fat or wax and the hydrogen peroxide above about 8.5.

After completion of the bleaching step, the products resulting from neutralization of the acid may be removed by any suitable procedure. They may be removed, for example, by washing the oil, fat or wax with acid or with acidulated water. Ordinarily this does not involve a step additional to those now employed, for as pointed out in German Patent 595,126, these products are customarily remelted or recovered over acidulated water at the conclusion of the bleaching process.

Oils, fats or waxes bleached in accordance with the process described will be observed to have a lighter color than those bleached under similar conditions but without the neutralization of free acid present by the addition of magnesium oxide or similar alkaline material. Moreover, it will be found that waxes, especially beeswax bleached in accordance with the procedure described, will be more satisfactory in that their desirable natural characteristics are less changed during the bleaching. Moreover, my improved process makes it possible to obtain more satisfactory and more uniform results, especially with those types of commercial waxes and beeswaxes which are exceedingly difficult to bleach to a satisfactory light color without substantially impairing their desired physical and chemical characteristics.

When bleaching substances which are more easily bleached by chemical agents, such as the readily bleachable varieties of beeswax, it has been found possible to eliminate the step of preliminary bleaching wherein the emulsified product is subjected to the action of an oxidizing agent. When this step is eliminated the bleaching is carried out in a single operation, the material to be bleached is in the liquid or in the molten state during this operation and, in general, a greater amount of hydrogen peroxide will be necessary than that necessary when the two-stage method is utilized. During the step of bleaching the oil, fat or wax in a single operation, the inorganic acids present should, of course, be neutralized by the addition to the reaction mixture of some material which is alkaline in reaction, more especially some material, preferably magnesium oxide, which meets the requisites previously given.

As examples of my improved process for the bleaching of oils, fats and waxes the following may be given:—

#### Example 1

A sample of Congo wax, a product especially

difficult to bleach, was first remelted in the usual manner as described in German Patent 595,126 over water containing hydrogen peroxide. This was a clarification and preliminary purification step.

The wax was then subjected to a preliminary bleaching step, by emulsifying the clarified and purified material with about twice its volume of hot water and a 4% solution of sodium peroxide. 10 Caustic soda in the amount of about 1% was also present. The amounts specified are by weight, based on the weight of the wax. In carrying out this step the sodium peroxide was first dissolved in about 20 times its volume of cold water, and 15 then gradually added to the wax emulsified in about twice its volume of hot water containing 1% of caustic soda. During this step the temperature was maintained sufficiently high to keep the wax in the molten condition. A temperature of 90-100° C. was found suitable.

After completion of this bleaching step, the time in which the bleaching was complete being observed by determining that point at which the active oxygen content of the bath became depleted, the emulsion was broken by the addition of a slight excess of dilute sulfuric acid. The wax was then clarified to as great an extent as possible by the introduction of steam and by permitting it to stand for a short period. The 30 lower aqueous layer was then drawn off, the wax being thus recovered.

Magnesium oxide in the amount of 0.1% based on the weight of the Congo wax, was then added. The wax was maintained in the molten state, the temperature being maintained between 35 90-100° C., and treated with a 4% solution of hydrogen peroxide (40% concentration). During this step the mixture was continuously stirred. When bleaching was complete, determined by 40 testing for residual oxygen, hot water was added to the wax and enough dilute sulfuric acid to dissolve the magnesium oxide. It was then allowed to stand for a period of time to effect clarification. The temperature was then lowered and the 45 wax permitted to solidify.

The wax bleached in this manner had a considerably lighted color than samples of wax bleached in the same general process but without 50 out the addition of magnesium oxide.

#### Example 2

A sample of Congo wax was bleached in accordance with the same process described in 55 Example 1 except that 0.1% of sodium bicarbonate ( $NaHCO_3$ ) was utilized in place of 0.1% magnesium oxide. The wax was clarified and lightened in color to substantially the same degree as

that obtained in accordance with the process of Example 1.

It should be understood that the various details of the general process described are intended to be illustrative and not restrictive except insofar as necessitated by the appended claims. As various changes may be made in the general procedure which I regard as my preferred embodiment without departing from the spirit and scope of my invention, the disclosure and description given herein, except as necessitated by the appended claims, are to be regarded as illustrative and in no sense limiting.

I claim:

1. A process of bleaching oils, fats and waxes 15 which comprises contacting the product to be bleached in the emulsified state with an oxidizing agent in order to effect a partial bleach, adding an acid thereto in amount sufficient to break said emulsion, adding to said product an alkaline 20 agent in amount sufficient to neutralize the free inorganic acid present, said amount not being in excess of that amount necessary to impart there- 25 to a pH of substantially 8.5, and then bleaching said product in the liquid or molten state with hydrogen peroxide under conditions wherein the mixture of said product and hydrogen peroxide is substantially neutral in reaction.

2. A process as defined in claim 1 wherein the 30 alkaline agent added for the purpose of neutralizing free inorganic acids present is magnesium oxide.

3. A process as described in claim 1 wherein the alkaline agent added is magnesium oxide in 35 amounts ranging from 0.1 to 0.2% based on the weight of said oil, fat or wax.

4. A process as defined in claim 1 wherein, at the conclusion of the hydrogen peroxide bleaching operation, the products formed by neutralization of the inorganic acids present with said 40 alkaline agent are removed by washing said oil, fat or wax with a dilute acid.

5. A process for bleaching oils, fats and waxes which comprises contacting the product to be bleached in the emulsified state with an oxidizing 45 agent in order to effect a partial bleach, adding an acid thereto in amount sufficient to break said emulsion, adding to said product an alkaline agent in amount sufficient to neutralize the free inorganic acid present therein but insufficient to 50 impart thereto a pH in excess of substantially 8.5, and then contacting said product in the liquid or molten state with hydrogen peroxide under conditions wherein the mixture of said product and hydrogen peroxide is substantially neutral in re- 55 action and remains substantially neutral throughout said final bleaching stage.

EMIL SCHELLER.